

C. P. STEINMETZ.  
ELECTRODE FOR ARC LIGHTS,  
APPLICATION FILED FEB. 26, 1902. RENEWED FEB. 26, 1904.  
**914,891.** Patented Mar. 9, 1909.



Contains Magnetite

Witnesses:  
Murray D. Badgley  
Glen A. Ford

Inventor:  
Charles P. Steinmetz  
By *Albert G. Davis*  
Atty.

# UNITED STATES PATENT OFFICE.

CHARLES P. STEINMETZ, OF SCHENECTADY, NEW YORK, ASSIGNOR TO GENERAL ELECTRIC COMPANY, A CORPORATION OF NEW YORK.

## ELECTRODE FOR ARC-LIGHTS.

No. 914,891.

Specification of Letters Patent. Patented March 9, 1909.

Application filed February 26, 1902, Serial No. 95,804. Renewed February 26, 1904. Serial No. 195,481.

To all whom it may concern:

Be it known that I, CHARLES P. STEINMETZ, a citizen of the United States, residing at Schenectady, in the county of Schenectady, State of New York, have invented certain new and useful Improvements in Electrodes for Arc-Lights, of which the following is a specification.

My present invention relates to improvements in electric arc lights and more especially to the composition of the terminals or electrodes used therein. When the terminals or electrodes are of carbon, as is now the common practice, the arc itself is of comparatively feeble intensity, the greater portion of the light being derived from the incandescent crater of the positive terminal. I have discovered however that if either or both of the terminals be made either in whole or in part of magnetite ( $Fe_3O_4$ ) instead of carbon, the arc assumes an entirely different character. Instead of being the minor factor in the production of light it becomes intensely luminous, giving off a brilliant white light with a spectrum like that of iron. If both electrodes or terminals are of magnetite it is immaterial which is positive and which is negative. If, however, one terminal be of carbon or of some substance other than magnetite, it is desirable that the magnetite terminal should be the negative. If, with one electrode of carbon and the other of magnetite, the polarity be reversed so that the magnetite is the positive terminal and the carbon the negative terminal, the arc instead of being of the luminous character mentioned, becomes dull and comparatively non-luminous and yellowish in color, the spectrum under these circumstances presenting bright sodium and potassium lines, showing the presence of these substances as impurities.

The use of magnetite for the purposes above described not only very greatly improves the quantity and character of the light, but possesses in addition the valuable feature that electrodes formed thereof waste away only very slowly, considerably slower in fact than the wasting away of correspond-

ing carbon electrodes. I find also that I may improve the action of the electrode by adding certain impurities such, for example, as magnesia, lime or alumina compounds or the like. In making the electrodes a suitable binding material may be used to render easier the formation of the electrodes out of its constituent material or materials.

In the accompanying drawing I have shown an electrode of the character in which my invention may be embodied.

What I claim as new and desire to secure by Letters Patent of the United States, is,—

1. An arc lamp electrode in which magnetite predominates.
2. An arc lamp electrode composed of magnetite.
3. An arc lamp electrode composed predominantly of a good conducting metallic oxid.
4. An arc lamp electrode composed predominantly of a metallic oxid of good conductivity and which when heated is but slightly attacked by air.
5. An arc lamp electrode which is a good conductor at ordinary temperatures, and contains a good conducting metallic oxid giving a luminous or flaming arc.
6. An arcing electrode composed essentially of an electrically conducting oxid.
7. An arcing electrode composed essentially of an oxid of iron.
8. An arcing electrode composed essentially of the magnetic oxid of iron.
9. An essentially metallic arcing electrode containing oxid of iron.
10. An essentially metallic arcing electrode containing magnetic oxid of iron.
11. An arc light electrode composed principally of magnetite.
12. An arc light electrode containing at least 75 per cent. of magnetite.

In witness whereof, I have hereunto set my hand this 24th day of February, 1902.

CHARLES P. STEINMETZ.

Witnesses:

HELEN ORFORD,  
ALEX. F. MACDONALD.